

Feb. 23, 1937.

A. W. DROBILE ET AL

2,071,922

MANUFACTURE OF PILE FABRICS

Filed July 19, 1934

4 Sheets-Sheet 1



Feb. 23, 1937.

A. W. DROBILE ET AL

2,071,922

## MANUFACTURE OF PILE FABRICS

Filed July 19, 1934

4 Sheets-Sheet 2



Feb. 23, 1937.

A. W. DROBILE ET AL

2,071,922

## MANUFACTURE OF PILE FABRICS

Filed July 19, 1934

4 Sheets-Sheet 3



INVENTOR.

Albert William Drobile,  
Glen Sefton Hiers and  
William Rollin Keen  
BY

BY *William Hollin Keen*

BY *William Hollin Neen*



100 ATTORNEY

ATTORNEY.

ATTORNEY.

Feb. 23, 1937.

A. W. DROBILE ET AL  
MANUFACTURE OF PILE FABRICS

2,071,922

Filed July 19, 1934

4 Sheets-Sheet 4

*Fig. 2.*



*Fig. 5.*



*Fig. 3.*



INVENTOR.  
Albert William Drobile,  
Glen Sefton Hiers and  
BY William Rollin Keen

*George W. Denney*  
ATTORNEY.

## UNITED STATES PATENT OFFICE

2,071,922

## MANUFACTURE OF PILE FABRICS

Albert William Drobile, Wayne, Glen Sefton Hiers,  
Bala-Cynwyd, and William Rollin Keen, Drexel  
Hill, Pa., assignors to Collins & Aikman Cor-  
poration, Philadelphia, Pa., a corporation of  
Delaware

Application July 19, 1934, Serial No. 735,922

35 Claims. (Cl. 26—1)

Our invention is an improvement in the manufacture of pile fabrics by which uniform products may be produced in a continuous operation at a maximum rate, at a minimum cost, and with 5 minimum loss from spoilage.

The dyeing and face treatment of pile fabrics after the weaving thereof have heretofore been uniformly practiced as batch operations, regardless of the quantity or volume of the product required, because the difficulties of continuous operations have been deemed insurmountable in 10 commercial production due to the great differences in the time involved in the various operations requisite for the conversion of fabric woven 15 wholly or partially in the gray into finished saleable fabrics.

We have found that by saturating a continuous length of pile fabric by movement thereof at a constant rate in momentary contact with a vehicle 20 containing a dyestuff having an exhaustion rate of not less than 2% during a contact period of fourteen-hundredths (14/100) of a minute, the fabric, after subjection to pressure, as by mangle, for forcing the dyestuff-containing vehicle into the fabric and for removal of excess vehicle and dyestuff, will have entrained therein 25 an amount of dyestuff unexhausted from the vehicle sufficient to give a desired tintorial effect, by the exhaustion of the dyestuff into and 30 fixation thereof in the fabric fibres during the passage of the fabric through a fixing or ageing atmosphere between the dyeing apparatus and the pile finishing apparatus, and hence the pile surface may be moved in contact with the pile 35 finishing devices at the same rate at which it was moved in contact with dyestuff-containing vehicle. Thus dyeing and finishing of continuous, 40 connected lengths of pile fabric may be concurrently carried on as a continuous operation.

The vehicle used is preferably an aqueous liquid containing dyestuff in much greater concentration than is permissible in kettle dyeing but insufficient in concentration to cause bronzing of 45 the dye on the pile tips or subsequent crocking of the dye, and the dye bath is maintained at a constant concentration, temperature, pH, and preferably level, with consequent constancy of the exhaustion rate of the dyestuff and entrainment thereof in the fabric, whose saturation is effected by one or more immersions in tensioned 50 condition in the bath and concurrent or subsequent passage of the fabric through nip rolls. To avoid bronzing and crocking and to supply material to the finishing apparatus at a rate 55 compatible with the permissible speed of finishing

operations, the immersion period should not be less than three-hundredths (3/100) of a minute and should not exceed two (2) minutes with the bath at a constant temperature between 180 and 210° F. Longer periods of immersion tend to 5 cause uneven dyeing and also cause concurrent immersion of excessive lengths of fabric which would be spoiled by any interruption in subsequent operations.

The dyestuff concentration, its rate of exhaustion, the bath temperature and the duration of immersion of the fabric therein must be maintained constant throughout a run to secure uniformity of shade or color after the passage of the first few yards through the bath, and such 10 condition of the dye bath is maintained by a uniform and continuous addition to the bath of 15 a rehabilitating mixture compensating for exhaustion, entrainment and evaporation therefrom.

A pile fabric may be run continuously through such a dye bath at a rate of from ten to eighteen yards per minute, and run through the pile finishing apparatus at substantially the same rate with a production of fabrics of improved color 20 and finish. The shade or color is uniform across the width and from end to end of the fabric, and a uniform coloration is also secured from the tips to the bases of the pile tufts. Our process 25 greatly decreases the amount of factory shrinkage as compared with kettle dyeing and batch finishing and substantially eliminates 30 creasing, matting, streaking, spotting, after dyeing and other difficulties incident to batch or intermittent production.

The continuity of our process of dyeing and 35 finishing renders it possible to match colors in the finished material without the difficulties incident to over-dyeing in a dye kettle during the period required for sampling, drying and conditioning a sample to regain its natural condition 40 for color matching and subsequent unloading.

Our invention is applicable to the manufacture 45 of pile fabrics composed entirely of vegetable fibres, such as cotton, or to the production of fabrics having a pile composed of animal fibre, such as mohair or wool, or partly of animal fibre and partly of vegetable fibre, and if desired, some of the yarns, as for instance, the backing yarns, may be dyed before weaving. Should the type 50 of tuft used or tightness of the backing be insufficient in themselves to prevent displacement of the pile tufts by the nip rolls or mangle, the pile may be more firmly anchored prior to dyeing by the permeation of the backing by aqueous 55

rubber or other solidifiable binder to form a layer within the backing, or by covering the bights of the pile loops by means of cover warps during weaving.

5 The dyes used having the characteristics hereinbefore set forth may be direct dyes, or neutral dyeing wool dyes, or other suitable dyestuffs may be used.

When the fabric contains both vegetable fibres and animal fibres, which fibres may be contained in the backing and pile respectively or may be both contained in the pile, and it is desired to dye both types of fibre simultaneously and continuously, the dye bath may contain a 10 dyestuff which will color uniformly the animal and vegetable fibres in so-called union effects. Or complementary dyestuffs may be used in the bath, one of which has a greater affinity for animal fibre than for vegetable fibre, and the other 15 of which has a greater affinity for vegetable fibre than for animal fibre. Appropriate selection may be made of direct dyestuffs having a greater affinity for animal fibre than for vegetable fibre and of other direct dyestuffs having a 20 greater affinity for vegetable fibre than for animal fibre, and by proper combinations of such dyestuffs similar or contrasting effects may be 25 simultaneously produced.

The several dyestuffs contained in the bath 30 should be selected and so proportioned therein and in the rehabilitating liquor added that the rates of exhaustion of the different dyestuffs are maintained substantially the same as one another and the concentration of each dyestuff is maintained substantially constant throughout the 35 period of operation.

In determining the relative rates of exhaustion in dyeing a union fabric containing animal fibre and vegetable fibre, the rate of exhaustion of the 40 neutral dyeing wool dyestuff is determined independently of the rate of exhaustion of the direct dyestuff, and from the data thus obtained the relative concentrations of the wool dyestuff and of the direct dyestuff in the rehabilitating liquor 45 may be calculated.

All of the dyestuffs used should be readily soluble, and should have a high tinctorial value.

Examples of neutral dyeing wool dyestuff colors which have been successfully used in the production 50 of commercially uniform plush fabrics in accordance with our invention are Alizarine Astrol B (Color Index No. 1075), Acid Anthraquinone Violet 3R (Color Index No. 1080), Kilton Fast Yellow 2GC (Color Index No. 636).

55 The wetting and saturation of the fabric in dyeing may be facilitated by the use of any of the known penetrants such as sulphonated oils, sulphonated alcohols, or naphthalenes or glyco products.

60 In the selection of dyestuffs for the union dyeing of fabrics containing both animal fibre and vegetable fibre in accordance with our process, it is desirable to avoid such dyestuffs as initially impart a deep stain to one type of fibre for which, 65 however, they have little or no lasting affinity and require continued agitation and boiling to level out from the fibre by which it is initially absorbed and impart a tinctorial effect to the other fibre. For instance, colors having an excessive initial affinity for and deep staining effect 70 on cotton, and little or no initial dyeing effect on wool, should be avoided for the dyeing of union fabrics.

If desired, the dyestuff vehicle may be of such 75 viscosity or may be so thickened by a water sol-

uble thickener as to form substantially a paste in which the dyestuff is so distributed as to secure uniform mechanical deposition on and subsequent uniform exhaustion into the fabric. Such vehicle may also contain salts capable of dissociation by heat or steam to release acid capable of reacting with the dyestuffs to promote exhaustion into and fixation of the dyestuff on the fabric fibres with which it contacts. 5

The dye-impregnated fabric passes, while still 10 moist, to an ager having a wet steam compartment in which such moisture and temperature conditions are maintained as result in substantially complete exhaustion of the dyestuff from the entrained vehicle, the deposition of such dyestuff in and upon the fibres and the development 15 and setting of the dye. The substantially exhausted entrained vehicle and any thickener contained therein is then washed from the fabric in a continuous rinsing or washing operation which 20 removes substantially all trace of free dyestuff. The fabric may then be after treated, as for instance, with acids or acidic materials, to improve the fastness of the dye, and, after rinsing, hydro-extraction, and wet tigering, if desired, is 25 dried in a suitable continuous dryer. The dried fabric leaving the dryer passes continuously, and at substantially the same rate at which it contacted with the dyestuff, through a range of synchronized pile finishing apparatus preferably 30 comprising sequentially arranged tigers, beaters, shears, brushes, humidifying apparatus, inspection and packaging apparatus.

The desired tinctorial effect of the dye upon 35 the fabric may be adjusted relatively to the rate of movement of the fabric in contact with the dye bath and through the pile finishing apparatus by—

(a) Varying the concentration of the dye-stuff in the dye vehicle; 40

(b) Varying the number of passes or duration of the immersion of the fabric in the dyestuff vehicle;

(c) Selection of dyestuffs of varying or different solubilities and rates of exhaustion; 45

(d) Varying the character and concentration of the chemical assists or wetting agents used;

(e) Varying the pH of the dyestuff-containing vehicle;

(f) Varying the degree and duration of the 50 pressure to which the fabric saturated with dye vehicle is subjected by the mangles or nip rolls;

(g) Varying the temperature of the dye bath;

(h) Varying the ageing time and conditions.

The sequence of steps and the characteristic 55 features and advantages of our improvements will further appear from the following description and the accompanying drawings in which—

Figs. 1a to 1f illustrate diagrammatically the contiguous sections of a range through which lengths of pile fabric connected by the stitching together of their ends to form a continuous strip are fed continuously at a constant rate through range dyeing and finishing equipment operated in synchronism to effect the movement of the fabric continuously at a constant rate of from ten to eighteen yards per minute and the production of a product which is consistently uniform after the first few yards of fabric have passed through the range; 60

Fig. 2 illustrates diagrammatically a detail of the nip rolls by which the fabric is squeezed to force the dyestuff-containing vehicle thereinto and the excess from the fabric; 70

Fig. 3 is a detail illustrating diagrammatically 75

a modified method and apparatus for impregnating the fabric with dyestuff;

Fig. 4 is a further detail illustrating diagrammatically a further method and apparatus for impregnating the fabric with dyestuff; and

Fig. 5 is a further detail illustrating diagrammatically a further method of and apparatus for impregnating the fabric with dyestuff dispersed in a thickened vehicle.

10 As an example by way of illustration only of the steps followed in a preferred practice of our invention, we have illustrated in Figs. 1a to 1f of the drawings the continuous feeding of a pile fabric A from a source of supply 1 to a dyeing apparatus 2 in which the fabric passes downwardly over guide rolls 3 and 4 into a trough 5 containing a bath of dyestuff dispersed in an aqueous vehicle. This bath is maintained at a constant temperature by heating coils 6 and is 15 maintained at a constant level by replenishment with a rehabilitating dye liquor supplied to the bath through a supply pipe 7 containing a control valve 8. The rehabilitating liquor is added to the bath substantially continuously and compensates 20 for absorption, exhaustion and evaporation and has a dyestuff concentration sufficient to maintain the dye bath substantially constant in its tintorial value. The pipe 7 is connected with a receptacle 9 provided with an overflow pipe 10 for 25 maintaining a constant level and pressure in the receptacle 9 which is supplied with the rehabilitating dye liquor from a mixing tank 11. The overflow through the pipe 10 may be collected in a tank 12 and returned to the mixing tank 11 by 30 a pump 13 and pipe 14. Preferably, the bath in the trough 5 is maintained at a constant temperature in the range from 180° to 210° and the pH value of the dye bath is controlled to maintain a constant exhaustion rate of the dyestuff of not 35 less than 2% nor more than 15% in a contact period of fourteen-hundredths (14/100) of a minute. In dyeing without the use of acidic assists, this may involve a pH range up to ten on the alkaline side and down to six on the acid side. 40 In acid dyeing, the pH value may vary from about 6 down to 4, depending upon the desired rate of exhaustion, temperature and period of contact or immersion. As an illustration of control utilized, when using the dyestuff known as Kiton Fast 45 Yellow 2GC (Color Index No. 636), the temperature of the bath is maintained constant at about 200° F. and with a pH value of approximately 9 to maintain an initial exhaustion rate of 2.34% in fourteen-hundredths (14/100) of a minute, 50 and for such time of immersion the rate of movement of the fabric is approximately 12½ yards per minute.

The volume of the bath is kept as small as is practicable while securing thorough admixture therewith of rehabilitating liquor and the thorough saturation of the fabric in passing therethrough.

The saturation may be effected in one or more immersions, and as illustrated, the fabric first 60 passes over the submerged journaled roller 15, is then squeezed between the rubber covered nip rollers 16 and 17, then passes over the submerged journaled roller 18 and is then again squeezed 65 between the rubber covered nip rollers 17 and 18 and between the rollers 18 and 19.

In passing through the bath and the rollers, the fabric is maintained in tension longitudinally or warp-wise and transversely or weft-wise.

In passing through the dye bath, the fabric A 75 is thoroughly saturated with the dye liquor which

is forced down to the bases of the pile tufts and into and through the backing or ground of the fabric by the squeezing action of the rolls 16, 17, 18 and 19. Any excess dye liquor expressed by the pressure of the rollers is returned to the dye trough 5. The repeated saturation of the fabric with the dyestuff-containing vehicle and the pressure applied thereto by the rollers 16, 17, 18 and 19 causes the entrained dyestuff-containing vehicle to thoroughly penetrate into the interstices 10 of the fabric and the pores of the fibres. The period of immersion of the fabric and the affinity of the dyestuff for its vehicle are such that the dyestuff is not completely exhausted into the fabric on leaving the nip rollers. The fabric 15 while still damp with its entrained dye liquor is passed to an ager 20 comprising a chamber containing wet steam through which the fabric is passed back and forth until the substantially 20 complete exhaustion of the dyestuff from the entrained dye liquor and the setting of the dyestuff in and upon the fibres of the fabric is finished. The temperature and saturation of the steam are so maintained and adjusted as to effect this 25 complete exhaustion and setting of the dyestuff during the period that the fabric is contained in the ager while moving forward therein continuously and at a constant rate.

The fabric while still damp, but with the dye 30 now firmly fixed, passes from the ager to a washing or rinsing machine 21 where any unfixed dye, thickener and dye vehicle is removed. The bulk of the moisture contained in the fabric when passing from the washer 21 is removed by suction applied to the fabric as it passes over the 35 mouth of the hydro-extractor 22.

Should it be desired to perform any other finishing operations on the fabric while it is still wet, these may be performed after the fabric 40 has left the first hydro-extractor 22. For instance, fabric may be moth-proofed or after-treated in the tank 23, have excess moisture removed by the hydro-extractor 22' and napped or the pile opened up while damp by passage 45 through the wet tigering machine 24.

When these operations, if performed, are completed, the fabric may be passed through a dew-drying machine 25' and then dried to substantially 50 its original area in the tenter drier 25 in which the fabric is stretched to substantially its original width by tenter chains 26 having thereon hooks 26' and by which the fabric is carried back and forth through the dryer while under tension warpwise and weftwise.

The dried fabric delivered from the dryer is 55 fed past the beater 27, through the brushing machine 28, dry tigering machine 29, and beater 30 to prepare the pile for shearing by the shear 31, after which the sheared plush is beaten and 60 brushed in the brushing machine 32 and may be 65 pressed by a steam press 33.

The fabric is now ready for the restoration of 70 its normal moisture content, which may be supplied thereto by a humidifier or conditioning machine 34 before the passage of the fabric to an inspection table 35 from which it passes to a roll-up and packaging machine 36.

While the fabric moves continuously and at a substantially constant rate from one unit to the next, it is preferable that there should be a certain amount of slack between the different units and to provide such slack the fabric may be pleated by folders 37 upon traveling conveyors 38 or delivered into J-boxes 39 conveniently positioned between some of or all of the machines. 75

As illustrated in Fig. 3, the pipe 7 may deliver the dye liquor into a pool enclosed by the contacting rollers 5a, 5b, 5c and 5d. With this arrangement the fabric A is passed between the 5 rubber covered rollers 5a and 5b and through the pool of dye liquor. The dye liquor is squeezed into the fabric and any excess dye liquor expelled therefrom by the passage of the fabric between the rollers 5a and 5c, around the roller 5c, and 10 between the rollers 5c and 5d. The fabric is then again saturated by passage through the pool and the dye liquor squeezed thereinto and any excess expelled therefrom by passage of the fabric between the rollers 5b and 5d.

15 As illustrated in Fig. 4, the tube 7 may discharge the dye liquor through a perforated section 7a onto the face of the fabric immediately in advance of the passage of the fabric between the rubber covered squeeze rolls 16' and 17' by 20 which the dye liquor is forced into the fabric and any excess squeezed therefrom.

As illustrated in Fig. 5, the dyestuff-containing vehicle may have the viscosity of, or be so thickened as to form, paste which is delivered through 25 suitable pipes 1' to the pool formed between the contacting rolls 39 and 40 and between the contacting rolls 41 and 42. The fabric A passes through the first pool of paste, then between the rolls 39 and 40, then through the second pool of 30 paste, and then between the rolls 41 and 42. The dyestuff-containing paste vehicle is thereby uniformly distributed over and forced into the fabric, which absorbs the dyestuff from the paste vehicle during the passage of the fabric through 35 the ager.

By each of these methods of applying the dyestuff to the fabric and exhausting dyestuff into the fabric after it has left the pool of dyestuff-containing vehicle, the fabric may be dyed at a 40 rate compatible with and permitting its finishing in a continuous operation during which the fabric is held in a tensioned condition during the performance thereon of operations tending to cause shrinkage.

45 When the manufacture of pile fabric requires the dyeing of both animal and vegetable fibres, or of cotton fibres alone, it is preferable that direct dyes or neutral wool dyes, or combinations thereof, be used in the practice of our process, but 50 where the cotton fibres are dyed prior to weaving and only wool or mohair fibres require dyeing, acid dyeing wool dyes may be used in the practice of our process by maintaining constant the acidity, temperature and volume or level of the 55 bath as well as the concentration and rate of exhaustion of the dyestuff.

In choosing between various dyestuffs for the practice of our process to produce a fabric of desired shade or color, there should be selected 60 readily soluble dyestuffs having a high tinctorial value at minimum concentration and which will disperse as true solutions or colloidal solutions in an aqueous vehicle instead of being merely mechanically suspended therein. The dyestuffs selected should be such as have exhaustion rates 65 within the limits hereinbefore specified and where two or more dyestuffs are used together they should exhaust at substantially the same rate under given conditions.

70 For example:

(a) Alazarine Supra Blue A (no Color Index number), a neutral dyeing wool color, has been used successfully with Pontamine Fast Yellow NNL (Color Index No. 814) a direct color.

75 (b) The direct color Pontamine Fast Yellow

NNL (Color Index No. 814) has been successfully used with the direct color Diamine Fast Brown R (no Color Index number).

(c) Neutral dyeing wool color, such as Alazarine Astrol B (blue) (Color Index No. 1075) has 5 been successfully used with Kiton Fast Yellow 2GC (Color Index No. 636), also a neutral dyeing wool color.

By rate or exhaustion or exhaustion rate, as used in the foregoing description and the appended claims, we refer to the ratio between—

(a) The weight of dyestuff which may be fixed in a given time of immersion on a given weight of textile from a dye bath of given concentration, temperature and pH, and

(b) The weight of dyestuff fixed on a similar quantity, quality and condition of textile when immersed in a dye bath under similar conditions temperature and at the pH employed and concentration required to produce the same shade 20 in the commonly used methods of dyeing with such dyestuff (for example in kettle dyeing with wool colors a pH equivalent to a concentration of .2 of 1% by-weight of commercial sulphuric acid and in kettle dyeing with direct or substantive color as pH equivalent to substantial neutrality) until practical exhaustion of the dyestuff has been reached.

Having described our invention, we claim:

1. In the manufacture of pile fabric, the steps 30 which include moving the pile fabric at a constant rate through a bath of dyestuff containing vehicle, entraining in the fabric a portion of such vehicle containing unexhausted dyestuff, exhausting the dyestuff from the vehicle and fixing the dyestuff on the fibers of the fabric in transit to pile finishing apparatus, and moving the fabric as a continuous web between and in contact with pile finishing devices in range.

2. In the manufacture of pile fabric, the steps 40 which include moving the pile fabric at a constant rate while contacting a dyestuff-containing vehicle, entraining in the fabric a portion of such vehicle containing unexhausted dyestuff, exhausting the dyestuff from the vehicle and fixing the dyestuff on the fibres of the fabric in transit to pile finishing apparatus, and moving the fabric in contact with pile finishing devices at substantially the rate at which the fabric moves in initially contacting with the dyestuff-containing vehicle.

3. In the manufacture of pile fabric, the steps 55 which include moving a pile fabric at a constant rate while momentarily contacting a supply of dyestuff-containing vehicle, squeezing said dyestuff-containing vehicle into said fabric and expressing the excess dyestuff-containing vehicle therefrom, the vehicle retained in said fabric containing unexhausted dyestuff, exhausting dyestuff from the vehicle into the fabric after said squeezing, washing the residual vehicle and unfixed dyestuff from the fabric, and finishing the pile of the fabric during movement thereof at substantially the rate at which it moved in contact with the dyestuff-containing vehicle supply.

4. In the manufacture of pile fabric, the steps 60 which include saturating a fabric with a dyestuff-containing vehicle during the movement of the fabric at a substantially constant rate, forcing into the fabric a portion of the dyestuff-containing vehicle, and expressing the remainder of such vehicle from the fabric, exhausting the dyestuff from the retained vehicle into the fabric while maintaining the fabric moist, removing the exhausted vehicle from the fabric, and shear-

15

25

25

35

45

50

55

60

65

65

70

75

ing the pile of the fabric during movement thereof at substantially the rate of movement thereof during saturation.

5. In the manufacture of pile fabric, the steps which include saturating the pile fabric with a dyestuff-containing vehicle during movement of the fabric at a substantially constant rate, forcing a portion of such saturating vehicle into the pores of the fabric fibres and expressing a portion of such vehicle from the fabric by pressure, exhausting dyestuff from the retained vehicle into the fabric and fixing it thereon while maintaining said fabric damp, removing the exhausted vehicle from the fabric, drying the 10 fabric, and tigering and shearing the pile while moving the fabric at a rate substantially the same as its rate of movement during saturation.

6. In the manufacture of pile fabric, the steps which consist in maintaining substantially constant the exhaustion rate in a dye bath containing a vehicle and having an exhaustion rate of at least 2% in fourteen-hundredths (14/100) of a minute contact with a pile fabric, moving a 15 pile fabric at a constant rate in momentary contact with said dye bath and entraining in the fabric such vehicle containing unexhausted dyestuff, forcing into the fabric a portion of such entrained vehicle, and expressing the remainder of such vehicle from the fabric, exhausting dyestuff from the retained vehicle into the fabric in an atmosphere of wet steam, removing the exhausted vehicle and any free dyestuff from the fabric, drying to reduce the moisture content below normal the fabric finishing the pile of 20 the fabric during the movement thereof at a rate substantially the same as its rate of movement during saturation, reconditioning the fabric uniformly by humidification and rolling up the fabric.

40 7. In the process set forth in claim 1, the step which consists in maintaining the exhaustion rate of the dyestuff from the bath substantially constant.

8. In the process set forth in claim 1, the steps 45 which consist in maintaining substantially constant the concentration of the dyestuff in the bath, the exhaustion rate of the dyestuff from the bath, and the temperature and pH of the combined dyestuff and vehicle.

50 9. In the process set forth in claim 2, the step which consists in maintaining substantially constant the volume of the supply of dyestuff-containing vehicle, and also maintaining substantially constant the concentration of dyestuff in 55 such vehicle and the rate of exhaustion of the dyestuff from the vehicle supply, and in maintaining substantially constant the temperature and pH of said supply of dyestuff-containing vehicle.

60 10. In the process set forth in claim 1, the steps which consist in maintaining in the vehicle bath a dyestuff having a primary affinity for animal fibre and a dyestuff having a primary affinity for vegetable fibre, and maintaining the 65 rates of exhaustion of said dyestuffs from the vehicle substantially uniform.

11. In the manufacture of pile fabrics containing animal and vegetable fibers according to claim 1, the steps which include maintaining 70 in the vehicle a neutral wool dyestuff and a direct dyestuff, maintaining the exhaustion rates of said dyestuffs substantially uniform.

12. In the manufacture of pile fabric containing animal fibre and vegetable fibre, the 75 steps which include passing such fabric at a

substantially constant rate through a dye bath having a substantially constant pH approximating neutrality, maintaining such bath at a substantially constant temperature and maintaining in such bath dyestuffs having exhaustion rates 5 for animal fibre and for vegetable fibre of not less than 2% in fourteen-hundredths of a minute.

13. In the manufacture of pile fabric, the steps which include saturating the pile and backing yarns of the fabric by passage of the fabric at a substantially constant rate through a dye liquor of constant temperature and constant dyestuff concentration for a period of immersion of not less than three-hundredths of a minute or in excess of two minutes, said dye liquor containing 15 dyestuff having an exhaustion rate of not less than 2% in fourteen-hundredths of a minute, removing from the fabric substantially all of the excess liquor, and exhausting from the fabric retained liquor after the removal of the excess 20 liquor sufficient dyestuff to give the fibres a desired shade upon fixation of the dyestuff therewith.

14. In the manufacture of pile fabric, the steps which include saturating a pile fabric by movement thereof at a substantially constant rate in contact with the dye liquor containing a dyestuff having a rate of exhaustion of at least 2% in 25 fourteen-hundredths of a minute of contact and requiring more than two minutes for substantially complete exhaustion of the actual dyeing constituent thereof, retaining in the fabric after emersion from the bath dye liquor containing unexhausted dyestuff, and substantially exhausting the dyestuff from retained dye liquor during 30 passage of the fabric from the dye bath to a pile finishing device.

15. In the manufacture of pile fabric which has been woven wholly or partly in the grey, the continuous steps which include moving the pile fabric at a constant rate while contacting a dyestuff containing vehicle for a time insufficient to completely fix the dye entrained by said contact, passing the fabric into a steaming atmosphere to more 40 completely fix the dye, washing the residual vehicle and unfixed dyestuff from the fabric, drying the fabric and rolling up the fabric.

16. In the manufacture of pile fabric which has been woven wholly or partly in the grey, the continuous steps which include moving the pile fabric at a constant rate while contacting a dyestuff containing vehicle for a time insufficient to completely fix the dye entrained by said contact, forcing the dyestuff containing vehicle uniformly 50 into the fabric and removing excess vehicle and dyestuff, passing the fabric into a steaming atmosphere to more completely fix the dye, washing the fabric to remove unfixed dye, thickener, and dye vehicle which may be in the fabric, drying the fabric to reduce the moisture content below normal 55 and rolling up the fabric.

17. In the manufacture of a pile fabric which has been woven wholly or partly in the grey, the continuous steps which include moving the pile fabric at a constant rate while contacting a 60 dyestuff containing vehicle for a time insufficient to completely fix the dye entrained by said contact, forcing the dyestuff vehicle uniformly into the fabric and removing excess vehicle and dyestuff, passing the fabric into a steaming atmosphere to more completely fix the dye, washing the fabric to remove unfixed dye, thickener or dye vehicle which may be in the fabric, extracting the water from the pile fabric which has been incorporated therein as a result of the washing, drying 65

the fabric to reduce the moisture content below normal and rolling up the fabric.

18. In the manufacture of a pile fabric which has been woven wholly or partly in the grey, the 5 continuous steps which include moving the pile fabric at a constant rate while contacting a dyestuff containing vehicle for a time insufficient to completely fix the dye entrained by said contact, forcing the dyestuff vehicle uniformly into the 10 fabric and removing excess vehicle and dyestuff, passing the fabric into a steaming atmosphere to more completely fix the dye, washing the fabric to remove unfixed dye, thickener or dye vehicle which may be in the fabric, extracting the water 15 from the pile fabric which has been incorporated therein as a result of the washing, subjecting this still damp fabric to a wet tigering operation to nap the pile and then drying the fabric to reduce the moisture content below normal and rolling up 20 the fabric.

19. In the manufacture of pile fabric which has been woven wholly or partly in the grey, the 25 continuous steps which include moving the pile fabric at a constant rate while contacting a dyestuff containing vehicle for a time insufficient to completely fix the dye entrained by said contact, forcing the dyestuff vehicle uniformly into the fabric and removing excess vehicle and dyestuff, 30 passing the fabric into a steaming atmosphere to more completely fix the dye, washing the fabric to remove unfixed dye, thickener or dye vehicle which may be in the fabric, extracting the water 35 from the pile fabric which has been incorporated therein as a result of the washing, after treating the fabric, extracting the surplus liquid incorporated in the fabric in the aftertreatment, subjecting the still damp fabric to a wet tigering operation to nap the pile, drying the fabric to reduce the moisture content below normal and rolling up 40 the fabric.

20. In the manufacture of a pile fabric which has been woven wholly or partly in the grey, the 45 continuous steps which include moving the pile fabric at a constant rate while contacting a dyestuff containing vehicle for a time insufficient to completely fix the dye entrained by said contact, forcing the dyestuff vehicle uniformly into the fabric and removing excess vehicle and dyestuff, 50 passing the fabric into a steaming atmosphere to more completely fix the dye, washing the fabric to remove unfixed dye, thickener or dye vehicle which may be in the fabric, extracting the water 55 from the pile fabric which has been incorporated therein as a result of the washing, mothproofing the fabric in a liquid bath, extracting the surplus liquid incorporated in the fabric by the mothproofer, subjecting the still damp fabric to a wet tigering operation to nap the pile, drying the fabric to reduce the moisture content below normal 60 and rolling up the fabric.

21. In the manufacture of a pile fabric which has been woven wholly or partly in the grey, the 65 continuous steps which include moving the pile fabric at a constant rate while contacting a dyestuff containing vehicle for a time insufficient to completely fix the dye entrained by said contact, forcing the dyestuff vehicle uniformly into the fabric and removing excess vehicle and dyestuff, 70 passing the fabric into a steaming atmosphere to more completely fix the dye, washing the fabric to remove unfixed dye, thickener or dye vehicle which may be in the fabric, extracting the water 75 from the pile fabric which has been incorporated therein as a result of passing through the washer, mothproofing the fabric in a liquid bath,

extracting the surplus liquid incorporated in the fabric by the mothproofer, subjecting the still damp fabric to a wet tigering operation to nap the pile, uniformly rewetting the fabric, drying the fabric to reduce the moisture content below 5 normal and rolling up the fabric.

22. In the manufacture of pile fabric which has been woven wholly or partly in the grey, the 10 continuous steps which include moving the pile fabric at a constant rate while contacting a dyestuff vehicle for a time insufficient to completely fix the dye entrained by said contact, passing the fabric into a steaming atmosphere to more completely fix the dye, washing the fabric to remove 15 unfixed dye, thickener or dye vehicle, drying the fabric to reduce the moisture content below normal, applying finishing operations to the pile and reconditioning the fabric by humidification and 20 rolling up the fabric.

23. In the manufacture of pile fabric which 25 has been woven wholly or partly in the grey, the continuous steps which include moving the pile fabric at a constant rate while contacting a dyestuff containing vehicle for a time insufficient to completely fix the dye entrained by said contact, forcing the 30 dyestuff containing vehicle uniformly into the fabric and removing excess vehicle and dyestuff, passing the fabric into a steaming atmosphere to more completely fix the dye, washing the fabric to remove unfixed dye, thickener or dye vehicle 35 which may be in the fabric, drying the fabric to reduce the moisture content below normal, applying finishing operations to the pile, reconditioning the fabric by humidification and 40 rolling up the fabric.

24. In the manufacture of pile fabric which has been woven wholly or partly in the grey, the 45 continuous steps which include moving the pile fabric at a constant rate while contacting a dyestuff vehicle for a time insufficient to completely fix the dye entrained by said contact, passing the fabric into a steaming atmosphere to more completely fix the dye, washing the fabric to remove unfixed dye, thickener or dye vehicle, drying the 50 fabric to reduce the moisture content below normal and reconditioning the fabric by humidification and 55 rolling up the fabric.

25. In the manufacture of pile fabric which has been woven wholly or partly in the grey, the 60 continuous steps which include moving the pile fabric at a constant rate while contacting a dyestuff containing vehicle for a time insufficient to completely fix the dye entrained by said contact, forcing the dyestuff containing vehicle uniformly into the fabric and removing excess vehicle and dyestuff, 65 passing the fabric into a steaming atmosphere to more completely fix the dye, washing the fabric to remove unfixed dye, thickener or dye vehicle which may be in the fabric, drying the fabric to 70 reduce the moisture content below normal, reconditioning the fabric by humidification and 75 rolling up the fabric.

26. In the manufacture of pile fabric, the steps 80 which include moving a pile fabric at a substantially constant rate while momentarily contacting a supply of dye-stuff-containing vehicle, entraining a portion of said vehicle in said fabric, squeezing said entrained dye-stuff-containing vehicle into said fabric after it has ceased to contact said supply, expressing the excess dye-stuff-containing vehicle therefrom, the vehicle retained in said fabric containing unexhausted dye-stuff, exhausting dyestuff from the vehicle into the fabric by passing said fabric while its pile is 85 still wet with the vehicle and flattened from the 90

- squeezing continuously through a heated humid atmosphere at a rate substantially the same as its rate of movement through said supply, straightening any mussed pile before the drying thereof, "setting" the straightened pile by drying the fabric under tension to a point below the normal moisture content of the fibres thereof, and restoring normal moisture content to the fabric.
- 5 27. In the manufacture of pile fabric, the steps which include moving a pile fabric at a substantially constant rate through a bath of dye-stuff-containing vehicle and entraining a portion of the vehicle therein, maintaining substantially constant the tinctorial value of said bath and the duration of immersion of sequential sections of fabric therein, squeezing the dye-stuff-containing vehicle into the sequential sections of fabric after they respectively leave the bath and 10 pressing excess dye-stuff-containing vehicle therefrom, the vehicle retained in the fabric containing unexhausted dyestuff, exhausting dyestuff from the vehicle into the fabric while the pile is still moist from the bath and flattened 15 from the squeezing, erecting any flattened pile before the "setting" thereof in flattened condition, and "setting" the erected pile by drying the fabric while tensioned.
- 25 28. In the manufacture of pile fabric, the steps which include moving a web of such fabric into and out of a bath of vehicle containing dyestuff having an exhaustion rate of not less than 2% during a contact period of 14/100 of a minute and which vehicle is entrained in the emergent 20 fabric without complete exhaustion therefrom of contained dyestuff, forcing the vehicle and dyestuff into the fabric by pressure tending to lay the pile in the same direction, exhausting dyestuff from the entrained vehicle into the fabric 25 by passage thereof through hot vapor while the fabric is still moist from the vehicle, washing any unexhausted dyestuff from the fabric, and drying the fabric.
- 30 29. In the manufacture of fabric as set forth in claim 28, the further step of straightening any mussed pile between the final exhaustion of the dyestuff and the drying of the fabric.
- 35 30. In the manufacture of fabric as set forth in claim 28, the step which includes drying the fabric below the normal moisture content of the fibres of the fabric, and humidifying the dried fabric to normal moisture content of the fibres.
- 40 31. In the manufacture of fabric as set forth in claim 28, the step which includes drying the fabric under tension and while stretched to approximately its original width.

32. In the manufacture of pile fabric, the steps which include moving a web containing tufts of resilient pile fibres into and out of a dyebath maintained at a substantially constant tinctorial value and having a temperature tending to plasticize the pile fibres, and at a rate entraining in the fabric unexhausted dyestuff, squeezing the dyestuff into the fabric by pressure tending to similarly lay the plasticized pile fibres, exhausting dyestuff into the fabric by 10 contact with heated vapor, straightening and erecting the plasticized pile fibres, dehydrating the fabric sufficiently to restore resilience to the pile fibres, and shearing the erected pile fibres.

33. In the manufacture of pile fabric, the steps which include passing a pile fabric as a substantially taut loop through a dye-bath maintained at a substantially constant tinctorial value, squeezing into the emergent fabric dyestuff entrained therein, exhausting dyestuff into 15 the fabric in transit after squeezing, washing unexhausted dyestuff from the fabric before the drying thereof, erecting the wet pile, the fabric being kept substantially free from pressure contacting laminations permitting migration of dyestuff from one section to another during the foregoing steps, drying the erected pile to a point below its normal moisture content, and humidifying the dried pile.

34. In the manufacture of pile fabric, the steps which include moving a pile fabric at a constant rate through a bath of dyestuff containing vehicle and moving such fabric at substantially the same rate in contact with pile finishing devices, the dyeing and the finishing 30 of the fabric being carried on as a continuous sequence of operation while maintaining in the vehicle bath a dyestuff having constantly an exhaustion rate from not less than 2% and not in excess of 15% in fourteen hundredths of a 35 minute contact with the pile fabric.

35. In the manufacture of pile fabric, the steps which include moving a pile fabric at a substantially constant rate through a bath of dyestuff containing vehicle and entraining a portion of the vehicle therein, forcing the entrained dyestuff vehicle into said fabric, removing the excess dyestuff vehicle therefrom, the vehicle retained in said fabric containing unexhausted dyestuff, exhausting the dyestuff 40 from the vehicle into the fabric in transit to pile finishing apparatus and moving the fabric in contact with pile finishing devices in range.

WILLIAM ROLLIN KEEN.

GLEN SEFTON HIERS.

ALBERT WILLIAM DROBILE.